

Aug. 23, 1960

M. B. VORDAHL

2,950,191

TITANIUM BASE ALLOYS

Original Filed Dec. 10, 1949



Fig.1



Fig.2



Fig.3

INVENTOR.  
MILTON B. VORDAHL  
BY   
John H. Lewis Jr.  
ATTORNEYS

1

2,950,191

## TITANIUM BASE ALLOYS

Milton B. Vordahl, Long Hill, Conn., assignor, by mesne assignments, to Crucible Steel Company of America, Borough of Flemington, N.J., a corporation of New Jersey

Filed May 31, 1951, Ser. No. 229,143

12 Claims. (Cl. 75—175.5)

This invention relates to the processing of alloys, particularly titanium-base alloys, and to alloys of a unique and desirable structure resulting from such processing.

In the drawings:

Fig. 1 is a photomicrograph of an alloy of commercial titanium with about 4.1% manganese after 90% work in the two-phase field.

Fig. 2 is a photomicrograph of an alloy of commercial titanium with about 6.8% manganese, the alloy having been extensively worked in the two-phase field, quenched from a temperature of 700° C., and stabilized at 500° C.

Fig. 3 is a partly theoretical phase diagram of the titanium-rich-end of the binary-titanium manganese system.

The low temperature or alpha phase of substantially pure titanium, which is of close-packed hexagonal structure, transforms at a temperature of about 885° C., to the high temperature or beta phase, which is of body centered cubic structure. The presence of such contaminants or alloying agents as carbon, oxygen and nitrogen, in the proportions in which they are commonly found in commercial titanium, tends to raise the beta transformation temperature, and establishes a relatively narrow zone or field of mixed alpha-beta structure. The presence of certain alloying metals, prominent among which are iron, chromium, manganese, and molybdenum, has a quite different effect upon transformation. Increasing amounts of these alloying materials stabilize the beta phase at progressively lower temperatures, and establish a mixed alpha-beta field of substantial scope. A typical phase diagram for an alloy of this type is shown in Fig. 3, the system selected for the purpose of illustration being the titanium-manganese system. The dotted lines represent probable boundaries which have not been exactly determined.

The present invention comprises the discovery of a method, believed to be unique in the metallurgical art, for securing an interleaved dispersion or distribution of two effectively stable and ductile phases, and of a unique structure resulting therefrom. An essential step in the method is the plastic deformation of the alloy at a temperature within the two-phase field. Another essential step is the selection of an alloy composition possessing two or more ductile phases stable over a suitable temperature range. Such plastic deformation of such a structure differs widely from the generally accepted practice of deforming to a desired size and configuration in a single phase field and subsequently heat treating to secure a desired set of properties. In the practice of applicant's method, the essentials of the desired structure are established by plastic deformation, and while subsequent heat treatment is permissible and may be further beneficial, it must be so controlled as not to destroy the essential structure set up by plastic deformation.

The alloys amenable to the present invention are of

2

the mixed-phase structure typified by the "alpha-plus-beta" field of the phase diagram, Fig. 3. They are characterized by the presence of two phases of unequal strength, both of which possess some ductility but which deform by basically different crystallographic mechanisms. Thus, a stress concentration in one phase tends to diffuse, rather than to propagate, when it encounters the other phase. The titanium base alloys particularly disclosed by this specification possess all of this unusual set of qualifications; their alpha phase is relatively weak but quite ductile; their beta phase is relatively strong while nevertheless maintaining some ductility; and alpha, being a hexagonal close-packed structure, deforms in a basically different manner than does beta, which has a body-centered-cubic structure.

The present invention is particularly directed to sheet, wire and rod products in which service stresses are applied substantially parallel to the rolling or drawing direction and in which, therefore, the optimum distribution of the weaker phase is in thin fibrils or platelets whose longitudinal axes are parallel to the rolling or drawing direction. The presence of the weaker phase in thin fibrils or platelets disposed parallel to the working direction presents a minimum area of weaker phase normal to the applied stress and so constitutes the strongest distribution; conventional processing procedures such as working in the all-beta region followed by cooling at any convenient rate produce a distribution of the weaker phase which presents an appreciably greater area of weaker phase normal to the applied stress than that achieved by the novel processing disclosed in this specification and so is weaker. A further important advantage of the optimum distribution is that a stress concentration arising in the stronger phase (which is making the major contribution to supporting the applied stress) tends, in starting to propagate across the fibrils and platelets of the weaker phase, to be diffused in a manner analogous to the reaction to stress of a cable in contrast to that of a rod.

Each of the phases in the optimum distribution disclosed by this specification may be either continuous or discontinuous in the worked direction. The stronger phase should predominate in order to give higher strength and thus tends to be continuous in the worked (and, therefore, the load-bearing) direction. Even if it is not continuous, however, its fibrils and platelets are coherent with their contiguous material and so, like the fibrils in a textile thread, act as if they were continuous. It is an essential feature of this invention that, normal to the direction of working, neither phase is continuous.

The history of the alloy prior to plastic deformation in a two-phase field is of little, if any, significance. The effect of plastic deformation in the two-phase field is to increase ductility at a given strength level, and this effect is quite independent of prior history. Whether the specimen had been hardened by quenching from a beta field or lower temperature or fully annealed by slow cooling from a beta field temperature or given any other treatment, extensive working in the two-phase field still develops its optimum properties, viz., the highest ductility at a given strength level. For example, the quenching from the all-beta field of a binary alloy of 4% manganese, balance substantially all commercial titanium, results in a structure characterized by extended martensite-like plates of alpha and irregular bodies of retained beta. The quenching from the all-beta field of a similar alloy containing about 7% manganese produces unstable beta grains. On subsequent elevated temperature aging or service there is a tendency to the growth of continuous bodies of alpha at the grain boundaries. Both structures are predisposed to fracture along the extended region of

relatively weak alpha. If either alloy is slow cooled it becomes "dead soft" and is, for most uses, in its least serviceable condition. Extensive two-phase working of either of these alloys from either the quenched or the annealed condition develops properties identical with those developed by working the same alloy from the other condition.

Extensive plastic deformation such as can be obtained in rolling sheet or rod or in drawing wire at a temperature within the two-phase field has the effect not only of breaking up and dispersing the continuous masses, particularly the relatively weak alpha, and reducing such continuous masses to much smaller, substantially discontinuous and discrete particles, but also of producing the interleaved structure of fibrils and platelets of alpha and beta which is disclosed by this specification as being optimum. If one phase predominates, it tends to form a matrix in which island platelets or fibrils of the second phase are embedded.

Fig. 1 is a photomicrograph at 600 magnification of a longitudinal section of a sheet of an alloy of commercial titanium with 4.1% manganese after a 90% area reduction by rolling at a temperature of 650° C., and stabilization for one hour at a temperature of 550° C. The lighter colored constituent is alpha titanium; the darker one is partially transformed beta. The dispersion and discontinuity of the phases, particularly the alpha phase, are very clear and are substantially optimum for sheet, a good balance being struck between properties transverse and parallel to the working direction. The platelets, which in the longitudinal section of Fig. 1 are shown edgewise, are arranged parallel to the sheet surfaces. In a wire, the fibrils would be arranged parallel to the axis, and the structure is comparable with that of a cable as compared with a solid rod. The individual fibers of the stronger but more brittle phase can, to some extent, yield separately and thus distribute the load throughout the whole, while the effect of stress-raising voids, lattice imperfections, and the like, tends to be nullified at the first junction with the weaker and more ductile phase.

A typical specimen of the 4.1% manganese alloy in the condition illustrated in Fig. 1 has a yield strength in excess of 120,000 p.s.i., an ultimate strength above 145,000 p.s.i., an elongation in  $\frac{1}{2}$ " of 16%, and a bend ductility of 3.3 T.<sup>1</sup> This ratio of ductility-to-strength is definitely superior to any obtainable from this alloy without extensive plastic deformation at a temperature within the two-phase field. The same is true of the numerous other alloys which have been found amenable to the processing of this invention. An alloy of 7% manganese, balance substantially all commercial titanium, after 75% area reduction by rolling at a temperature of 650° C., shows a structure substantially similar to that of the 4.1% manganese alloy illustrated in Fig. 1. Prior to such warm working and after furnace cooling from 750° C., it showed a heterogeneous mass of variously oriented extended bodies of the two phases. After 75% warm rolling and stabilization for one hour at 550° C., alloys of commercial titanium with about 8% manganese show a yield strength of about 145,000 p.s.i., an ultimate strength over 157,000 p.s.i., an elongation in  $\frac{1}{2}$ " of about 16%, and an average bend ductility of about 3 T.

While the broad invention contemplates plastic deformation at any temperature within the two-phase field at which the strength of the alloy permits such deformation, the working temperature should not too closely approach the boundary temperature between the mixed alpha-beta field and the beta field. The heating of the alloy prior to working, and possibly local heating in-

duced by working itself promote transformations toward equilibrium at the particular temperature. If the working temperature is too close to the all-beta temperature, the tendency to beta formation is so great that a substantial part of the benefits of the invention may be lost. In general, the working temperature should not approach the all-beta temperature within about 100 centigrade degrees.

Increasing amounts of plastic deformation within the two-phase field effect increasingly complete dispersion and interleaving of the phases, and proportionately increase ductility at a given strength level. Generally stated, strength is a function of composition and conditions of stabilization subsequent to two-phase temperature working. For an alloy of given composition, it has been found possible, by appropriate stabilization, to maintain a substantially constant strength-level throughout varying amounts of plastic deformation. Any material variations in strength being thus eliminated, the progressive increase in ductility with increasing two-phase temperature deformation has been established, without complication by other variables. The experimental work leading to the present invention was exhaustive, comprising different alloys, different treatments prior to two-phase working, different working temperatures, and varying amounts of two-phase temperature deformation.

As an example of the work, the following series of tests is described. Three alloys were selected which contained, respectively, 3.5%, 4.1% and 4.7% manganese, balance substantially all commercial titanium. An ingot of each composition was forged at 870° C. to a  $\frac{1}{2}$ " to  $\frac{5}{8}$ " slab, each slab was cleaned and rolled at about 815° C., to sheet of four different thicknesses so chosen that the varying amounts of warm rolling reduction (to be described) resulted in specimens of the same thickness, i.e., all finished specimens received the same total reduction from the ingot. Each of the twelve sheets was subdivided into three parts, and the three parts respectively of each sheet were conditioned for two-phase temperature rolling by three different treatments, as follows:

Condition "Q"—Heated in air one hour at 815° C., water quenched;  
 Condition "Q-T"—Heated in air one hour at 815° C., water quenched, and tempered sixteen hours at 550° C.;  
 Condition "F-C"—Heated in air one hour at 815° C., furnace cooled.

All specimens were then rolled to a uniform thickness at a two-phase field temperature, three different temperatures being used. The thickest specimens of each set were reduced 90%, the next thinner 75%, the next thinner 60%, and the thinnest 30%, the final rolled thickness of all being the same. All specimens were then stabilized for one hour at 550° C. Strength and ductility were then measured, and found to be as follows:

Composition: 3.5% manganese—balance, commercial titanium.  
 Rolling temperature: 650° C.  
 Stabilized: 1 hour at 550° C. after rolling.

| Pre-Rolling Condition | Reduction, percent | Yield (1,000s p.s.i.) | Ultimate (1,000s p.s.i.) | Percent Elongation | Bend Ductility (Least Favorable Direction) |
|-----------------------|--------------------|-----------------------|--------------------------|--------------------|--------------------------------------------|
| Q-----                | 30                 | 107                   | 136                      | 15                 | 7.7                                        |
| Q-----                | 60                 | 106                   | 134                      | 19                 | 5.1                                        |
| Q-----                | 75                 | 102                   | 130                      | 20                 | 3.1                                        |
| Q-----                | 90                 | 103                   | 130                      | 21                 | 2.6                                        |
| Q-T-----              | 30                 | 102                   | 131                      | 17                 | 9.0                                        |
| Q-T-----              | 60                 | 100                   | 131                      | 19                 | 4.3                                        |
| Q-T-----              | 75                 | 96                    | 126                      | 21                 | 2.5                                        |
| Q-T-----              | 90                 | 99                    | 125                      | 23                 | 2.6                                        |
| F-C-----              | 30                 | 102                   | 131                      | 16                 | 6.3                                        |
| F-C-----              | 60                 | 100                   | 130                      | 19                 | 3.7                                        |
| F-C-----              | 75                 | 98                    | 126                      | 21                 | 3.1                                        |
| F-C-----              | 90                 | 100                   | 124                      | 23                 | 3.1                                        |

<sup>1</sup>(The measurement of bend ductility is not standardized. The present applicant and his associates measure this property as the radius over which the specimen can be bent to an angle of 75° without cracking, the radius being expressed as a multiple of specimen thickness.)

Composition: 4.7% manganese—balance, commercial titanium.  
Rolling temperature: 700° C.  
Stabilized: 1 hour at 550° C. after rolling.

| Pre-Rolling Condition | Reduction, percent | Yield (1,000s p.s.i.) | Ultimate (1,000s p.s.i.) | Percent Elongation | Bend Ductility (Least Favorable Direction) |
|-----------------------|--------------------|-----------------------|--------------------------|--------------------|--------------------------------------------|
| Q-----                | 30                 | 119                   | 137                      | 8                  | 10                                         |
| Q-----                | 60                 | 128                   | 141                      | 6                  | 10                                         |
| Q-----                | 75                 | 121                   | 136                      | 17                 | 6.4                                        |
| Q-----                | 90                 | 112                   | 132                      | 19                 | 3.1                                        |
| Q-T-----              | 30                 | 124                   | 138                      | -----              | 10                                         |
| Q-T-----              | 60                 | 124                   | 137                      | 6                  | 6.2                                        |
| Q-T-----              | 75                 | 121                   | 136                      | 9                  | 3.4                                        |
| Q-T-----              | 90                 | 111                   | 132                      | 21                 | 2.3                                        |
| F-C-----              | 30                 | 110                   | 134                      | 6                  | 6.6                                        |
| F-C-----              | 60                 | 115                   | 138                      | 13                 | 6.6                                        |
| F-C-----              | 75                 | 111                   | 135                      | 16                 | 3.1                                        |
| F-C-----              | 90                 | 113                   | 135                      | 17                 | 2.3                                        |

Composition: 4.1% manganese—balance, commercial titanium.  
Rolling temperature: 555° C.  
Stabilized: 1 hour at 550° C. after rolling.

| Pre-Rolling Condition | Reduction, percent | Yield (1,000s p.s.i.) | Ultimate (1,000s p.s.i.) | Percent Elongation | Bend Ductility (Least Favorable Direction) |
|-----------------------|--------------------|-----------------------|--------------------------|--------------------|--------------------------------------------|
| Q-----                | 30                 | 117                   | 140                      | 3                  | 10                                         |
| Q-----                | 60                 | 130                   | 144                      | 3                  | 10                                         |
| Q-----                | 75                 | 128                   | 141                      | 7                  | 7.6                                        |
| Q-----                | 90                 | 125                   | 139                      | 12                 | 6.2                                        |
| Q-T-----              | 30                 | 110                   | 138                      | 4                  | 10                                         |
| Q-T-----              | 60                 | 114                   | 135                      | 12                 | 7.8                                        |
| Q-T-----              | 75                 | 119                   | 134                      | 14                 | 6.4                                        |
| Q-T-----              | 90                 | 123                   | 134                      | 18                 | 3.8                                        |
| F-C-----              | 30                 | 107                   | 132                      | 6                  | 10                                         |
| F-C-----              | 60                 | 111                   | 134                      | 12                 | 6.4                                        |
| F-C-----              | 75                 | 109                   | 132                      | 14                 | 4.6                                        |
| F-C-----              | 90                 | 113                   | 132                      | 18                 | 3.9                                        |

The temperature of 815° C., to which all of the alloys were heated prior to the two-phase rolling, if not within the all-beta field lies so close to the all-beta field as to destroy the effect of previous working. The tabulated results definitely show for each alloy rolled from each of three pre-rolling conditions, first, a negligible variation in yield and ultimate strength with varying amounts of

two-phase temperature rolling; and, second, a progressive increase in ductility for increasing amounts of such rolling. These effects are the same at any of the three rolling temperatures. Other variables being eliminated, increasing amounts of plastic deformation in the two-phase field effect a progressive increase in ductility.

Stabilization, as above described, is desirable under most conditions, and can be performed at temperatures up to about 550° C., without materially altering the microstructure typified by Fig. 1.

While the optimum combination of strength and ductility is secured by extensive plastic deformation in the two-phase field, fabrication problems frequently render it impossible to roll sheet to the strength level desired in the fabricated product. Bending, forming, drilling, and like operations, cannot be satisfactorily performed at the desired high strength. It has been found that the alloys processed according to the present invention can be annealed to the low strength level necessary for fabrication, and, after fabrication, quenched to the desired high strength, and still retain the essentials of the dispersed phase structure. The alpha phase is spheroidized, but remains as discrete bodies rather than continuous masses.

Fig. 2 is a photomicrograph of an alloy containing 6.8% manganese, balance commercial titanium, which, after extensive plastic deformation in the two-phase field, had been heated for 1 hour at 700° C., and water quenched; it will be seen to consist of a beta matrix containing very numerous relatively small and substantially discrete globules of alpha. This specimen, after stabilization for 1 hour at 500° C., showed a yield strength of about 140,000 p.s.i., an ultimate strength of about 170,000 p.s.i., and elongation in  $\frac{1}{2}$ " of about 12%, and a bend ductility of about 3 T.

While in the foregoing description the binary alloys of titanium and manganese have been used for the purpose of illustration, it has been found as the result of very extensive work that the novel processing is equally applicable to any alloys comprising two ductile phases, both of which are relatively stable at normal temperatures. Prominent among these are the binary alloys of titanium with molybdenum, chromium and iron, as well as manganese; and the ternary and higher alloys of titanium with

| Composition (Balance Titanium) | Tensile Properties |          |                               |             |                          |          |                               |             |     |
|--------------------------------|--------------------|----------|-------------------------------|-------------|--------------------------|----------|-------------------------------|-------------|-----|
|                                | As Warm Rolled     |          |                               |             | As Stabilized at 600° C. |          |                               |             |     |
|                                | 0.2% Yield         | Ultimate | Elongation in $\frac{1}{2}$ " | Bend Radius | 0.2% Yield               | Ultimate | Elongation in $\frac{1}{2}$ " | Bend Radius |     |
| Mn 3.4                         | C 0.23             | 51,000   | 76,000                        | 21          | 0.8                      | 138,000  | 149,000                       | 18          | 3.3 |
| Mn 4.4                         | C 0.22<br>N 0.1    | 152,000  | 173,000                       | 12          | 6.5                      | 144,000  | 160,000                       | 22          | 4.9 |
| Mn 6.1                         | C 0.12<br>N 0.03   | 159,000  | 184,000                       | 13          | 6.5                      | 132,000  | 146,000                       | 12          | 2.9 |
| Mn 13.2                        | C 0.15             | 170,000  | 187,000                       | 2           | 6.2                      | 155,000  | 160,000                       | 12          | 4.0 |
| Cr* 7.4                        | C 0.34             | 134,000  | 154,000                       | 7           | 4.6                      | 132,000  | 143,000                       | 14          | 2.7 |
| Cr* 12.4                       | C 0.17             | 141,000  | 160,000                       | 5           | 7.0                      | 133,000  | 142,000                       | 11          | 2.7 |
| Fe 2.4                         | C 0.32<br>N 0.02   | 117,000  | 146,000                       | 12          | 2.7                      | 98,000   | 125,000                       | 19          | 1.7 |
| Fe 5.0                         | C 0.25             | 138,000  | 164,000                       | 8           | 8.8                      | 119,000  | 141,000                       | 8           | 6.5 |
| Mo 4.7                         | C 0.2<br>N 0.1     | 135,000  | 159,000                       | 16          | 7.5                      | 122,000  | 145,000                       | 20          | 6.2 |
| Mn 3.4                         | C 0.51             | 140,000  | 170,000                       | 8           | 6.1                      | 135,000  | 159,000                       | 10          | 5.8 |
| Al 2.8                         | N 0.01             | 127,000  | 154,000                       | 14          | 4.8                      | 117,000  | 134,000                       | 21          | 2.0 |
| Mn 3.1                         | C 0.11<br>N 0.03   | 127,000  | 154,000                       | 10          | 6.5                      | 127,000  | 139,000                       | 19          | 2.7 |
| Al 4.1                         | C 0.32             | 136,000  | 164,000                       | 6           | 5.2                      | 117,000  | 134,000                       | 22          | 3.0 |
| Mn 3.4                         | C 0.32             | 127,000  | 153,000                       | 4           | 7.5                      | 138,000  | 150,000                       | 20          | 6.6 |
| Mo 0.8                         | N 0.03             | 153,000  | 171,000                       | 6           | 7.3                      | 148,000  | 158,000                       | 13          | 6.2 |
| Mn 3.2                         | C 0.09<br>N 0.02   | 127,000  | 153,000                       | 5.7         | 118,000                  | 138,000  | 15                            | 2.2         |     |
| Cr 1.9                         | C 0.2              | 155,000  | 175,000                       | 10          | 6.5                      | 149,000  | 160,000                       | 14          | 4.4 |
| Mn 2.5                         | N 0.02             | 127,000  | 158,000                       | 10          | 5.7                      | 118,000  | 138,000                       | 15          | 2.2 |
| Fe 1.6                         | C 0.32             | 155,000  | 178,000                       | 4           | 7.5                      | 149,000  | 160,000                       | 14          | 4.4 |
| Mn 5.5                         | C 0.32             | 153,000  | 171,000                       | 6           | 7.3                      | 148,000  | 158,000                       | 13          | 6.2 |
| Al 1.0                         | C 0.32             | 153,000  | 171,000                       | 6           | 7.3                      | 148,000  | 158,000                       | 13          | 6.2 |
| Cr 6.1                         | C 0.42             | 153,000  | 171,000                       | 6           | 7.3                      | 148,000  | 158,000                       | 13          | 6.2 |
| Mn 6.0                         | C 0.2              | 127,000  | 158,000                       | 10          | 5.7                      | 118,000  | 138,000                       | 15          | 2.2 |
| Cr 4.3                         | N 0.02             | 127,000  | 158,000                       | 10          | 5.7                      | 118,000  | 138,000                       | 15          | 2.2 |
| Mn 3.3                         | C 0.2              | 127,000  | 158,000                       | 10          | 5.7                      | 118,000  | 138,000                       | 15          | 2.2 |
| Fe 1.0                         | N 0.02             | 127,000  | 158,000                       | 10          | 5.7                      | 118,000  | 138,000                       | 15          | 2.2 |
| Al 4.0                         |                    |          |                               |             |                          |          |                               |             |     |

\* Stabilized at 700° C.

various metals of this group. Likewise included are the ternary and higher alloys of titanium with the metals of this group, and with aluminum. While in the binary titanium-aluminum alloys the beta phase is not stable at normal temperatures, it is stabilized by the addition of one or more of the metals, manganese, molybdenum, chromium and iron. The weight percentages of the different metals of the group, manganese, molybdenum, chromium and iron, which, when added to titanium produce a two-phase structure, vary with the particular metal—the maximum for manganese, for example, being about 13%, but the atomic percentages fall within the range of about 2 to about 15 atomic percent. Below about 2 atomic percent the beta phase is either absent altogether or present only in a negligible amount; while above about 15 atomic percent the alloys show an all-beta structure. Typical alloys and their properties as worked in the two-phase field, both with and without subsequent stabilization, are shown in the preceding table.

The present invention is believed to be of broad scope in that a desired structure having desired properties is secured by plastic deformation in the two-phase field, and not by any heat treating sequence of an article which has been fabricated to a desired form by deformation in a single-phase field with little if any regard to the properties desired in the finished article. While the examples in the foregoing specification are all from two-phase systems, the method is obviously applicable to systems containing more than two phases, all of which possess the requisite stability and ductility.

This application is a division of applicant's prior co-pending application, Serial No. 132,327, filed December 10, 1949, now abandoned.

What is claimed is:

1. An improved titanium base alloy which contains about 1 to 4% iron, up to about .30% maximum of each of the gases oxygen and nitrogen, and at least two metals within the ranges specified from the group consisting of: chromium about .5 to 6%, manganese about .5 to 6%, and molybdenum about .5 to 5%; the iron-plus-alloying metal content being less than 10% but not less than about 5%; the alloy being characterized by its good ductility and impact strength with relatively high tensile strength.

2. An improved titanium base alloy as defined in claim 1 as heat treated by working above and within its alpha-beta phase range of about 1800° to 1000° F., followed by annealing in a lower portion of its alpha-beta region of about 900° to 1400° F., and wherein its structure has alpha islands in a matrix of retained beta.

3. An improved titanium base alloy as defined in claim 1 as treated by rapidly cooling it from an upper portion to slightly above its alpha-beta phase range of about 1400° to 1800° F., followed by reheating to the lower portion of such range, about 900° to 1400° F., and wherein its structure has alpha islands in a matrix of retained beta.

4. An improved titanium base alloy which contains about 1 to 4% iron, up to about .30% maximum of each of the gases oxygen and nitrogen, at least two metals within the ranges specified from the group consisting of: chromium about .5 to 5%, manganese about .5 to 6%, and molybdenum about .5 to 5%, the iron-plus-alloying metal content being less than 10% but not less than about 5%, and the balance titanium with incidental impurities.

5. An improved titanium base alloy which contains about 1 to 4% iron, up to about .30% maximum of each of the gases oxygen and nitrogen, about 1 to 6% chro-

mium, about 1 to 5% molybdenum, the iron-plus-alloying metal content being less than 10% but not less than about 5%, and the balance titanium with incidental impurities.

6. An improved titanium base alloy which contains about 2 to 3.5% iron, up to about .20% maximum oxygen and about .15% maximum nitrogen, about 2 to 5% chromium, about 1.5 to 4.5% molybdenum, the iron-plus-alloying metal content being less than 10% but not less than 5%, and the balance titanium with incidental impurities.

7. An improved titanium base alloy which contains about 1 to 3% iron, up to about .30% maximum of each of the gases oxygen and nitrogen, about 1 to 6% of chromium, about 1 to 5% manganese, the iron-plus-alloying metal content being less than 10% but not less than about 5%, and the balance titanium with incidental impurities.

8. An improved titanium base alloy which contains about 1.5 to 2.5% iron, up to about .20% maximum oxygen and about .15% maximum nitrogen, about 2 to 4% chromium, about 2 to 4.5% manganese, the iron-plus-alloying metal content being less than 10% but not less than about 5%, and the balance titanium with incidental impurities.

9. An improved titanium base alloy which contains about 1 to 4% iron, up to about .30% maximum of each of the gases oxygen and nitrogen, about 1 to 5% molybdenum, about 1 to 6% manganese, the iron-plus-alloying metal content being less than 10% but not less than about 5%, and the balance titanium with incidental impurities.

10. An improved titanium base alloy which contains about 1.5 to 3% iron, up to about .20% maximum oxygen and about .15% maximum nitrogen, about 1.5 to 4% molybdenum, about 2 to 4.5% manganese, the iron-plus-alloying metal content being less than 10% but not less than about 5%, and the balance titanium with incidental impurities.

11. An improved titanium base alloy which contains about 1 to 4% iron, up to about .30% maximum of each of the gases oxygen and nitrogen, about .5 to 5% chromium, about .5 to 5% molybdenum, about .5 to 6% manganese, the iron-plus-alloying metal content being less than 10% but not less than about 5%, and the balance titanium with incidental impurities.

12. An improved titanium base alloy which contains about 1.5 to 3.5% iron, up to about .20% maximum oxygen and about .15% maximum nitrogen, about 1.5 to 3.5% each of chromium and manganese, about 1 to 3% molybdenum, the iron-plus-alloying metal content being less than 10% but not less than about 5%, and the balance titanium with incidental impurities.

#### References Cited in the file of this patent

#### UNITED STATES PATENTS

|           |               |               |
|-----------|---------------|---------------|
| 2,205,854 | Kroll         | June 25, 1940 |
| 2,554,031 | Jaffee et al. | May 22, 1951  |
| 2,588,007 | Jaffee        | Mar. 4, 1952  |
| 2,640,773 | Pitler et al. | June 2, 1953  |

#### FOREIGN PATENTS

|         |         |               |
|---------|---------|---------------|
| 718,822 | Germany | Mar. 24, 1942 |
|---------|---------|---------------|

#### OTHER REFERENCES

"Zeitschrift fur Metallkunde," vol. 29 (1937), pages 190 and 191.

"Transactions of the American Institute of Mining and Metallurgical Engineers," vol. 166 (1946), pages 390-396.

UNITED STATES PATENT OFFICE  
CERTIFICATE OF CORRECTION

Patent No. 2,950,191

August 23, 1960

Milton B. Vordahl

It is hereby certified that error appears in the printed specification of the above numbered patent requiring correction and that the said Letters Patent should read as corrected below.

Column 8, line 10, for "50%" read -- 5% --.

Signed and sealed this 11th day of April 1961.

(SEAL)

Attest:

ERNEST W. SWIDER

Attesting Officer

ARTHUR W. CROCKER  
Acting Commissioner of Patents